

May 13, 1930.

L. W. TARR

1,758,867

TRACK INSULATION

Filed Feb. 23, 1929



Fig. 2.

Fig. 3.



BY *Nester W. Tarr* <sup>Inventor</sup>  
*E. C. Brandenburg*  
*Attorney*

## UNITED STATES PATENT OFFICE

LESTER W. TARR, OF NEWARK, DELAWARE, ASSIGNOR, BY MESNE ASSIGNMENTS, TO  
CONTINENTAL-DIAMOND FIBRE COMPANY, OF NEWARK, DELAWARE, A CORPOR-  
ATION OF DELAWARE

## TRACK INSULATION

Application filed February 23, 1929. Serial No. 342,273.

This invention relates to an improvement in track insulation.

Vulcanized fibre has been used very largely for insulation in the case of railway signal systems. It is a tough material which fulfills certain requirements but it is not satisfactory because of the troubles which occur from the fibre becoming wet under atmospheric conditions, which renders it a conductor of electric current instead of an insulator.

To overcome this difficulty the present invention utilizes a material for track insulation that will not absorb moisture appreciably when it becomes wet and which therefore cannot act as a conductor under such conditions. This material may be a laminated fibrous material, which is completely saturated throughout with a phenolic condensation product, such as bakelite, which product saturates all of the fibres of the material so that there could be no possibility of the absorption of moisture in appreciable quantities, and therefore no possibility of lessening the insulating qualities of the material when it becomes wet.

The material may be used alone or combined with vulcanized fibre. Its combination with vulcanized fibre strengthens and toughens the insulation considerably, thereby preventing it from becoming stiff and subject to fracture. This combination is effected preferably in layers secured together in a suitable manner and shaped to form the desired track insulation.

In the accompanying drawings:

Fig. 1 is a sectional view through a portion of a railway rail with the insulation applied thereto;

Fig. 2 is a sectional view through a modification of the arrangement of materials in the insulation;

Fig. 3 is a similar view showing a further modification; and

Fig. 4 is a perspective view of the insulation.

The numeral 1 designates the rail, on one or both sides of which the insulation is to be applied. The insulation is designated generally by the numeral 2 and is adapted to be secured to the web portion of the rail where

it is held by the usual bolts, which hold the rail ends together.

The web of the rail is usually filled up with a wooden piece so as to make the joint perfectly rectangular on the inside. The insulation is illustrated as being of three layers, although it may be of only two if desired, the layers being placed face to face and secured together by cementing by bakelite water-glass or some other satisfactory adhesive agent. This may be accomplished during the molding operation if desired.

The layers might also be riveted together.

In Fig. 1, the fibrous insulating material is designated by the numeral 3, it being on the opposite sides of vulcanized fibrous material 4 and secured thereto to form a sheet from which is molded or otherwise formed the proper shape of the track insulation. This insulating material is of suitable fibre, such as paper or canvas, completely saturated throughout with a phenolic condensation product, such as bakelite, which extends to all of the fibres of the material in order that they will be completely saturated and to prevent any appreciable absorption of moisture, which might possibly act to turn the material into a conductor instead of an insulator, which is very objectionable and undesirable.

The vulcanized fiber is a tough material and used to prevent fracture of the insulating material.

In Fig. 2, the vulcanized fibre or toughening material is located on opposite sides of the insulating fibrous material, which is the reverse of the arrangement shown in Fig. 1. In Fig. 3, the insulating material is shown on the inside with the vulcanized fibre outside, or this arrangement may be reversed in the two-ply material, which is illustrated in Fig. 3. The insulation may be either of two or three-ply and the insulating material may be either inside or outside of the vulcanized fibre but these are secured together as a unit. The insulating material serves to insulate the rails effectively while the vulcanized fibre that is used in connection therewith acts to overcome the brittleness that may be characteristic of some of the in-

sulating material, rendering it free from fracture.

The insulating material used is of any suitable fibrous nature, such as canvas or paper or other similar material that is completely saturated throughout with a phenolic condensation product, such as bakelite, which saturates all of the fibres of the material, rendering them impervious to moisture, preventing the absorption of moisture and rendering the insulation free from any conducting properties, even under extremely wet atmospheric conditions.

I claim:

- 15 1. A rail insulation formed of fibrous material saturated with a phenolic condensation product, and a fibrous insulating backing material secured thereto.
- 20 2. A rail insulation comprising a layer of fibrous material saturated throughout with a phenolic condensation product, and a layer of fibrous insulating backing material integrally secured thereto to prevent fracture of the insulating material.
- 25 3. A rail insulation comprising a layer of fibrous insulating material having all of the fibres thereof completely saturated with a phenolic condensation product, and a layer of vulcanized fibrous material secured to a face thereof to prevent fracture of the insulating material.
- 30 4. A rail insulation comprising a layer of fibrous insulating material saturated throughout with a phenolic condensation product, and a layer of vulcanized fibrous material permanently attached to the surface thereof to strengthen said insulating material.
- 35 5. A rail insulation comprising a layer of fibrous insulation material having all of the fibres thereof completely saturated with a phenolic condensation product, and a layer of vulcanized fibrous material permanently attached to the surface thereof as a unit to strengthen said insulating material.

In testimony whereof I affix my signature.

LESTER W. TARR.